

## UNITED STATES PATENT OFFICE

2,400,563

FILLED ASPHALT AND ASPHALT COATED  
ROOFING COMPOSITIONS

Francis L. Mark, Redondo Beach, Calif.

No Drawing. Application October 5, 1942,  
Serial No. 460,920

4 Claims. (Cl. 106—281)

This invention relates to filled asphaltic cements and to filled asphaltic coating composition employing balanced mixtures of finely divided mineral matter, such as fine mineral dust, and diatomaceous earths. Filled asphalt containing mineral dust, such as rock dust and diatomaceous earths have been employed during the past for various uses. It has been observed that the addition of diatomaceous earth to steam refined asphalt has the effect of imparting to such asphalt some of the properties of air-blown asphalt, the addition of the diatomaceous earth increasing the softening point and lowering the penetration of steam refined asphalt. The addition of diatomaceous earth also has the effect of increasing the tensile strength of steam refined asphalt. However, such mixtures of asphalt and diatomaceous earth do not have the pliability of air-blown asphalt mixtures and at low temperatures are brittle. This brittleness of such asphalts has excluded them from use in one of the most important fields of asphalt application, that is in prepared roofing.

Prepared roofing, whether of the rolled sheet type or the shingle type, is prepared by saturating felted material with a saturating asphalt, after which the asphalt saturated sheet is coated with a filled type asphalt material. The coated asphalt may be sprinkled with rock granules while the asphalt is soft and the granules are pressed into the asphalt.

The type of asphalt which has been employed for this coating purpose has been an air-blown asphalt because the steam blown asphalts, even though they are filled, are too brittle at low temperatures and too soft at high temperatures. Fillers are employed in the asphalt for the purpose of stiffening the asphalt and rendering it less susceptible to temperature change. The mineral fillers, which have been used in the past, consist of pulverized limestone or other rock dust, fine silica sand, ground mica, talc, ground asbestos, slate flour and the like. While this type of coating has shown good utility, it has imposed certain serious limitations upon the temperature to which the roofing may be exposed in construction or use. One of the most serious of these difficulties is the cracking or shattering of the asphalt at low temperatures. Thus the asphalt coated roofing may not be laid at temperatures much below about 50° to 60° F. Shingles when laid at this temperature are shattered when nails are driven through the shingles. Rolled roofing is wound into rolls usually on a mandrel core of 4" to 5" 55

in diameter. When this roll is unwound at low temperatures transverse cracks appear in the coating and often carry clear through the base felt itself. As a result, the roofing cap sheet disintegrates and allows water to enter the underlying roof structure. This may result in leaks and in moisture blisters on the surface.

In order to limit this cold weather cracking it has been necessary in the past to use relatively soft asphalts. This was made particularly imperative by the fact that the filler added to the asphalt had the effect of actually increasing the brittleness of the asphalt. The manufacturer of asphalt roofing was then on the horns of a dilemma. He could have asphaltic roofing which would not run and excessively soften at the high temperatures to which the roofing might be exposed in the summertime by using an asphalt of a relatively high melting point and adding sufficient filler and as a result suffer the cracks and shattering effect which follow from the brittleness of such mixtures at low temperatures. He could use a soft asphalt and limit his filler content to obtain proper pliability at low temperatures, but suffer the consequences of a running asphalt at high temperatures. Since such asphalts at high temperatures become displaced when asphalt roofings are positioned at any angle and since the granules of aggregate employed as a coating become displaced, due to the softness of the asphalt, such asphalt roofings are impractical.

Since the latter considerations are more important and in many cases controlling, the manufacturer was forced to suffer the consequences of lack of low temperature pliability of his filled asphalt type of coating.

I have now made the discovery that diatomaceous earth when used in proportioned mixes with mineral dust in oxidized asphalt gives a balanced mix which removes the manufacturer from the horns of the dilemma. It gives the high temperature stability together with the low temperature pliability.

Diatomaceous earth, as employed in this invention, produces a marked increase in the softening point of the asphalt. Less than ten per cent of this material when used with mineral dust in proper proportion will raise the softening point of a blown asphalt from about 195° F. to 230° F., resulting in a coating of greatly improved pliability and higher tensile strength and resistance to displacement and running at high temperatures. The effect of diatomaceous earth in increasing

the pliability of the asphalt has permitted me to make roofing material which may be handled as low as 5° F. without any cracking. In unrolling such a rolled roofing no cracking has been apparent, even down to the last portion with sharpest curvature. Repeated flexing of this material has shown that it is entirely pliable so that it may be handled without cracking. When using this material on shingles it may be nailed at temperatures well below freezing without shattering.

Asphalt roofing may contain small amounts of water even though the asphalt is carried to 500° F. in its preparation. It is present due to absorption in the felted sheet and may be present under the roofing laid over an old roof or it may enter through seams. When this moisture expands into vapor it causes blistering of the surface and a destruction of the coating. I have found that the addition of this diatomaceous earth in proper proportion, mixed with mineral filler material gives a tougher surface which prevents blistering. This arises from the fact that the diatomaceous earth will increase the tensile strength of the asphalt.

The ability of the diatomaceous earth to raise the melting point while improving the low temperature pliability has permitted me to use lower softening point oxidized asphalts and thus I have been able to improve the adhesive properties of the asphalt for the granules employed in coating the asphalt. Whereas in the prior practice it has been found necessary to use relatively high softening point asphalts in order to overcome the softening effects of high temperature, I have been enabled to use relatively low softening point asphalts because I have been able to impart this high temperature stability by the use of diatomaceous earth. This lower softening point has improved the adhesive properties of the asphalt mix and I have been able to overcome the tendency of the asphalt to run and the granules to be displaced at high temperatures.

The diatomaceous earth also results in a filled asphalt of improved weathering properties when subjected to the standard "Weatherometer" test in which the asphalt was subject to ultra-violet rays at 140° F. and frozen at 10° F. in repeated operations. The diatomaceous earth filled asphalts of my invention show an improvement in weathering characteristics showing a resistance to failure of one-third or more. In other words, they may be exposed to the above treatment for a 33 1/3% greater period than the rock dust filled type of oxidized asphalt before failure occurs.

The following example of one embodiment of my invention is given by way of illustration and not for the purpose of limiting my invention:

In making the filled asphalt of my invention, I employ an air-blown asphalt having a ball and ring softening point of 190° to 205° F. The asphalt is heated to a temperature of about 350° or higher, sufficient to impart fluidity to the asphalt. To this asphalt is added mineral filler of the conventional type, to-wit: rock dust, pulverized limestone, fine silica sand, ground mica, talc, volcanic ash, clays, ground asbestos, powdered shells, slate flour. Diatomaceous earth is also added. I find that I obtain superior results by first dispersing the diatomaceous earth in the asphalt, agitating the mixture to ensure dispersal and to free mixture of water. The mineral filler is then added. The diatomaceous earth has the effect of supporting the mineral filler to prevent undue settling. I prefer, but I am not limited,

to use kiln dried diatomaceous earth that is uncalcined material having a water content of about 6% or less. For best results, diatomaceous earth should have a wet density of about 18 or less pounds per cubic foot. I may, however, use material having a wet density from 13 to 22 or other diatomaceous earths. By wet density is meant that density determined by the conventional test in which one gram of the diatomaceous earth is suspended in distilled water in a 15 centimeter centrifuge tube which is filled to the 15 centimeter mark. The tube is whirled at 1800 revolutions per minute and the volume occupied by the diatomaceous earth is read and converted into pounds per cubic foot.

The asphalt and diatomaceous earth and powdered mineral filler are proportioned to give the following properties. The ball and ring melting point should be 210° F. or better. The viscosity of the mixture when read at 360° by the "Brookfield Viscosimeter" should be in the range of about 5,000 to 20,000 centipoises. The penetration, when measured on the standard penetrometer, according to ASTM specifications, employing 100 grams for five seconds at 77° F. should range from about 1.2 to 1.7 millimeters. I proportion the asphalt, rock dust, and diatomaceous earth to obtain the above specifications. While other proportions and specifications will give a useful result and I do not desire to be limited to the illustration of my preferred embodiment, I have found that the above limits give a highly advantageous result when employed as a coating for rolled roofing.

In the following table, which illustrates various examples of compositions employed, the symbol S. P. represents the softening point of the asphalt. The symbol P. D. represents paving dust and D represents diatomaceous earth and B. & R. stands for ball and ring softening point.

|                    | 55% of 195 S. P. | 62% of 195 S. P. |
|--------------------|------------------|------------------|
| % Filler           | 39% P. D., 6% D. | 8% D., 30% P. D. |
| Softening point    | 230              | 219              |
| Penetration—77° F. | 1.7              | 1.7              |
| Vis. at 360°       | 9,200 C. P.      | 5,000 C. P.      |

Table 1

| Percent asphalt | Percent diatomaceous earth | Percent paving dust | Softening point (B. & R.) | Penetration 77° |
|-----------------|----------------------------|---------------------|---------------------------|-----------------|
| 100             | —                          | —                   | 195                       | 26              |
| 55              | 7.5                        | 37.4                | 229                       | 16              |
| 55              | 6                          | 39                  | 228                       | 16              |

Table 2

In choosing the diatomaceous earth to be employed in my composition, I have discovered that by a proper selection of the type of diatoms which I use I have been able to obtain a highly improved result in increasing the melting point and tensile strength as well as the pliability of filled asphalt. This improvement in these properties is of general utility in filled asphalts employing diatomaceous earth, such as in pipe line coating, road construction and in all places where filled asphalt has been employed as an asphaltic cement. There are over 10,000 different types of diatoms. Of these types there is one class of diatoms which is termed the elongated type.

The type of diatoms which are here referred to are those whose length is markedly greater than their width. The round or disc shaped diatoms, known as the "discus" species, including also those of square or oblong cross-section which have

their dimensions of length and width nearly equal, do not have as great an effect. This type of diatom may be employed, but must be used in larger amounts nor do they have the effect of improving the low temperature pliability and the tensile strength that is obtained with the elongated type. These elongated forms are characterized by skeletons which are wide and thin or long and narrow. These elongated diatoms are to be contrasted with the small heavy walled type. 10 This classification is well understood in this art. See 1, 2, 3, and 9, and 12 to 18 of "Diatomaceous Earth by Calvert, A. C. S. Monogram Series 52, Edition of 1930." Some examples of the elongated type appear in Fig. 16. Examples of the 15 round type appear in Fig. 13. I have found that when employing these elongated diatoms I may obtain a better result in improvement of tensile strength and low temperature pliability than when employing diatoms whose dimensions of 20 length and breadth more closely approach each other, as in the case of the round type of diatom.

It is to be understood that the foregoing examples are for purposes of illustration and are not to be considered as limiting of the invention. Various changes and modifications may be made therein without departing from the spirit of the appended claims.

I claim:

1. A filled asphalt comprising an oxidized asphalt having a ball and ring softening point of about 190° to about 205° F. and mineral filler and kiln dried diatomaceous earth whose diatoms, in preponderant proportion, are of the elongated type, having a wet density of less than about 30 18, said mixture of asphalt, filler, and diatomaceous earth having a ball and ring softening point of at least 210° F., and higher than said oxidized asphalt, a viscosity of about 5,000 to 20,000 centipoises at 360° F. and a penetration of 1.2 to 1.7 millimeters when measured at 77° F., employing 100-gram weight for five seconds.

2. A filled asphalt comprising an oxidized asphalt having a ball and ring softening point of about 190° to about 205° F. and mineral filler and kiln dried diatomaceous earth having less than about 6% moisture, said mixture of asphalt, 5 filler and diatomaceous earth, whose diatoms in preponderant proportion are of the elongated type, having a ball and ring softening point of at least 210° F. and higher than said oxidized asphalt, a viscosity of about 5,000 to 20,000 centipoises at 360° F. and a penetration of 1.2 to 1.7 millimeters when measured at 77° F., employing 100-gram weight for five seconds.

3. Prepared roofing comprising sheet material 15 coated with a filled asphalt comprising an oxidized asphalt having a ball and ring softening point of about 190° to about 205° F. and mineral filler and kiln dried diatomaceous earth whose diatoms, in preponderant proportions, are of the elongated species, having a wet density of less than about 18, said mixture of asphalt, filler and diatomaceous earth having a ball and ring softening point of 210° F. or better, and higher than said oxidized asphalt, a viscosity of about 5,000 to 20,000 centipoises at 360° F. and a penetration of 1.2 to 1.7 millimeters when measured at 77° F., employing 100-gram weight for five seconds.

4. Prepared roofing comprising sheet material 20 coated with a filled asphalt comprising an oxidized asphalt having a ball and ring softening point of about 190° to about 205° F. and mineral filler and kiln dried diatomaceous earth whose diatoms, in preponderant proportions, are of elongated species, having less than about 6% moisture, said mixture of asphalt, filler and diatomaceous earth having a ball and ring softening point of 210° F. or better, and higher than said oxidized asphalt, a viscosity of about 5,000 to 20,000 centipoises at 360° F. and a penetration of 25 1.2 to 1.7 millimeters when measured at 77° F., employing 100-gram weight for five seconds.

FRANCIS L. MARK.